

# UNITED STATES PATENT OFFICE.

LOUIS S. ROSS, OF NEWTONVILLE, MASSACHUSETTS.

## RAILWAY TIME-BURNING SIGNAL-FUSEE.

1,025,883.

Specification of Letters Patent.

Patented May 7, 1912.

No Drawing.

Application filed February 15, 1912. Serial No. 677,852.

*To all whom it may concern:*

Be it known that I, LOUIS S. ROSS, a citizen of the United States, and a resident of Newtonville, in the county of Middlesex and 5 State of Massachusetts, have invented an Improvement in Railway Time-Burning Signal-Fusees, of which the following description is a specification.

This invention relates to improvements in 10 time burning railway signal fusees, the primary object thereof being to produce a fusee for such purpose that will not spontaneously ignite under conditions to which it is necessarily subjected, and which will not be 15 extinguished when thrown from a moving train or otherwise subjected to severe shock, and which insures continuity of the flame after lighting.

In most compositions for railway signal 20 fusees produced prior to my invention, there have been certain recognized characteristics of the ingredients contained in the fusees that render the latter extremely susceptible to spontaneous ignition, particu- 25 larly in the presence of heat or moisture.

The railways of the United States for a number of years past have maintained a 30 bureau for the safe transportation of explosives and other dangerous articles. This bureau employs chemists to investigate 35 questions relating to the manufacture of explosives and other dangerous articles, and from time to time makes regulations and issues specifications prescribing the inherent characteristics of time burning railway signal fusees. These regulations must be 40 passed upon and approved by the Interstate Commerce Commission to render them legally binding and effective. In accordance 45 with the requirements of the said bureau, railway signal fusees comprise a paper tube of heavy, tough fiber, in which the composition is packed, carrying at one end a spike adapted to penetrate the railway ties or bed 50 and having at its opposite end means for igniting the fusee.

Railway signal fusees are usually thrown 55 from the rear of a moving train and are necessarily therefore subjected to rough usage. It is therefore necessary to have the paper tube of sufficient strength to withstand this usage without breakage. These fusee paper tubes are therefore made of heavy, tough fiber, as stated, and the rail-

roads require that the finished fusee must 55 stand a specified, relatively heavy weight at its center when supported at its ends. One of the tests of the said bureau is that the fusee after burning a number of seconds in air must burn a specified time when completely submerged in water. It is further required by the said bureau that the fusee must burn a predetermined specified length of time. It must burn with brilliancy and 60 force of flame and it must burn under either favorable or unfavorable weather conditions. In other words, the railway signal fusee must burn in strong winds or storms or even in pools of water or snowbanks.

By reason of the necessity of burning the 70 tube in uniformity with the burning of the composition and also of the necessity that the composition burn with force and brilliancy, all successful compositions for railway signal fusees heretofore employed have 75 contained sulfur and potassium chlorate as fundamental ingredients, with the single exception that a perchlorate, preferably perchlorate of potassium, has been substituted for the chlorate in a composition containing 80 sulfur.

For many years it has been known that time burning railway signal fusees containing sulfur and potassium chlorate as heretofore combined were subject to spontaneous 85 ignition and combustion due to climatic conditions of heat and moisture, because of the presence of said ingredients in the composition, and attempts have been made for many years by railway chemists 90 and others to overcome this serious defect. Such spontaneous ignition has been attributed to the production by sulfur in the presence of heat and moisture of sulfurous and sulfuric acids, which in the presence of 95 potassium chlorate decompose the latter and generate chlorin peroxid. The formation of sulfuric acid from sulfur requires the presence of oxygen, which is readily obtained in the breaking up of the potassium 100 chlorate, whereby heat is generated, accelerating and helping to continue the reaction until a condition is reached that produces spontaneous combustion.

The so-called chlorate time burning rail- 105 way signal fusee is composed of chlorate, sulfur, carbohydrate and metallic nitrate in suitable proportions. In order to overcome

the tendency to spontaneous ignition characteristic of the chlorate fusee, a so-called perchlorate fusee has been made by substituting perchlorate of potassium for the chlorate of potassium.

5 A fusee made of mixtures containing a perchlorate, such as perchlorate of potassium, is recognized to be harder to ignite and more easily extinguished when thrown 10 from a moving train than a fusee of the so-called chlorate type. The so-called perchlorate fusee, in spite of this objection, is used because of its substantial freedom from spontaneous ignition.

15 Because of the fact that a perchlorate fusee is substantially free from danger of spontaneous ignition, I have conducted a series of experiments in order to produce if possible a perchlorate fusee that will not be 20 readily extinguished by sudden shock and the flame of which will burn with continuity. I have as the result of said experiments discovered that if a relatively short portion of the fusee at the igniting end contain 25 an excess quantity of sulfur or perchlorate, and preferably perchlorate, that such fusee when ignited will burn with excessive or extreme force and rapidity until said short portion is consumed and that 30 thereafter the fusee will continue to burn with normal force and rapidity, because then in a quiescent condition.

The remaining portion of the fusee is 35 preferably composed wholly of ingredients in normal proportion, because if it contain the indicated increased percentage of potassium perchlorate or even of sulfur, it will burn with such rapidity and force as to be consumed before the expiration of the time 40 interval during which the fusee should burn. Moreover the indicated excessive percentage of perchlorate if continued throughout the fusee would render the cost of the fusee prohibitive.

45 Perchlorate fusees as heretofore manufactured usually contain from five or six to twenty per cent. of potassium or other perchlorate combined with which are nitrate, sulfur and carbohydrate, with charcoal and 50 antimony if desired, in substantially the following proportions:—nitrate 50 to 95%, sulfur 3 to 23%, carbohydrate 1 to 11%, charcoal 1%, antimony 1%.

By suitably increasing either the sulfur 55 or the perchlorate, and by which latter I mean either potassium perchlorate or any other suitable perchlorate, such for example as ammonium perchlorate, and preferably by increasing the perchlorate from the five 60 or six to twenty per cent. heretofore used to about fifteen to thirty per cent., I have succeeded in producing a fusee which is free from danger of spontaneous ignition, and which cannot be readily extinguished by 65 sudden shock. In other words, I have ob-

tained a fusee having the combined advantages of the perchlorate and of the chlorate fusee.

The length of that portion of the fusee containing the excessive quantity of perchlorate of potassium or other ingredient 70 may be varied within the scope of my invention and may and preferably does vary with the diameter of the fusee, and also in some cases will vary with variations in the 75 total length of the fusee. Preferably, however, I make such portion of the fusee long enough to occupy about one minute in burning. In other words, I have obtained excellent results by making such portion of 80 the fusee containing an excessive quantity of perchlorate or sulfur about one inch in length.

In certain cases, fusees are held in the trainman's hand for a considerable period 85 as a torch signal and immediately thereafter are thrown to the ground. Therefore, that portion of the fusee containing the excessive proportion of perchlorate or sulfur should be long enough to insure the burning 90 of the fusee with increased force and rapidity until after the fusee has been so thrown to the ground.

In accordance with my invention, I preferably provide, as customary in the so-called perchlorate fusee, a suitable mixture of perchlorate (preferably perchlorate or potassium) though I may employ any suitable perchlorate, sulfur, carbohydrate or carbonaceous material and a metallic salt, such 10 as a metallic nitrate or oxid, to which, if desired, I may add charcoal and antimony. The perchlorate of potassium is used to furnish the principal supply of oxygen, the sulfur mainly to increase combustion, the 105 carbohydrate or carbonaceous material to furnish carbon and hydrogen to aid combustion and to smooth and deepen the flame, and the metallic salt, preferably that of strontium, barium or sodium to constitute 110 the base or coloring ingredients. While the proportions of these ingredients may be varied, they are preferably those previously stated. The carbonaceous material preferably employed by me consists of rosin or 115 red gum, charcoal and sawdust and grease in suitable proportions.

The increased proportion of the perchlorate of potassium in the described portion of the fusee at the igniting end may be varied 120 within the scope of my invention, but I have obtained best results by employing about thirty per cent. of perchlorate of potassium in said portion of the fusee.

Inasmuch as that portion of the fusee 125 containing the excessive proportion of perchlorate will cause such portion of the fusee to burn with excessive or extreme force and rapidly, I preferably reinforce that part of the fusee tube or casing that surrounds or 130

contains the described portion of the fusee composition. This I do in order to prevent the burning away too quickly of this portion of the fusee tube or casing. This result I best effect by providing a short supplemental paper or other case placed either inside of outside the fusee case at the igniting end, such supplemental case being preferably of a length substantially corresponding to the length of that portion of the fusee containing the excessive quantity of perchlorate. The provision of this supplemental case enforces a slight chimneying, which does not continue after the flame has reached that portion of the fusee containing the normal proportion of ingredients, and therefore is not objectionable. This enforced chimneying is of advantage, as it prevents too rapid burning away of the fusee case at the igniting end.

The fusee case may be otherwise constructed as usual, and is preferably provided with a handle or spike at one end and with any suitable igniting means at the other end.

In defining the fusee as provided at the igniting end with an excess quantity of perchlorate or sulfur, I include constructions wherein the portion of the fusee containing such excess quantity does not extend to the very igniting tip of the fusee, but terminates more or less short thereof. By providing the described excess quantity at the igniting end, that is, at or more or less near the extreme igniting tip, I provide means whereby the fusee is not extinguished when thrown, even though it be held in the hand for a more or less short interval after lighting and before throwing.

It will be evident from the foregoing description that a fireworks compound such as a railway fusee signal constructed in accordance with my invention possesses the marked advantage of the perchlorate fusee in that it is substantially free from liability to spontaneous ignition, and that it is free from all tendency to be readily extinguished from sudden shock. In other words, a fusee constructed in accordance with my invention will burn under all adverse conditions.

Having thus described one embodiment of my invention and the best manner known to me for carrying the same into effect, I desire it to be understood that the scope of the invention is set forth in the following claims.

Claims.

1. A time burning railway signal fusee containing sulfur and a perchlorate, a short portion of said fusee at the igniting end having both of said ingredients commingled, one of said ingredients being contained therein in excess, thereby to cause the burning of said portion with excessive or abnormal force and rapidity, and the remainder
2. A time burning railway signal fusee containing sulfur and a perchlorate, a short portion of said fusee at the igniting end having both of said ingredients commingled, said perchlorate being contained therein in excess, thereby to cause the burning of said portion with excessive or abnormal force and rapidity, and the remainder of said fusee having said ingredients normally proportioned, thereby to burn with less force and rapidity. 70
3. A time burning railway signal fusee containing metallic nitrate, sulfur and perchlorate of potassium, a short portion of said fusee at the igniting end having said ingredients commingled, at least one of said latter two ingredients being contained therein in excess, thereby to cause the burning of said portion with excessive or abnormal force and rapidity, and the remainder of said fusee having said ingredients normally proportioned, thereby to burn with less force and rapidity. 80
4. A time burning railway signal fusee comprising a metallic nitrate, a carbonaceous material, sulfur, and a perchlorate, a short portion of said fusee at the igniting end having said ingredients commingled, at least one of said latter two ingredients being contained therein in excess, thereby to cause the burning of said portion with excessive or abnormal force and rapidity, and the remainder of said fusee having said ingredients normally proportioned, thereby to burn with less force and rapidity. 90
5. A time burning railway signal fusee comprising a metallic nitrate, sulfur, a carbohydrate and a perchlorate, a short portion of said fusee at the igniting end having sulfur and perchlorate commingled, said perchlorate being contained therein in excess, thereby to cause the burning of said portion with excessive or abnormal force and rapidity, and the remainder of said fusee having said ingredients normally proportioned, thereby to burn with less force and rapidity. 100
6. A time burning railway signal fusee containing metallic nitrate, sulfur, a carbohydrate and perchlorate of potassium, a short portion of said fusee at the igniting end having sulfur and perchlorate of potassium commingled, said perchlorate of potassium being contained therein in excess, thereby to cause the burning of said portion with excessive or abnormal force and rapidity, and the remainder of said fusee having said ingredients normally proportioned, thereby to burn with less force and rapidity. 110
7. A time burning railway signal fusee containing sulfur and a perchlorate, said fusee having two sections both containing said ingredients in commingled condition, 120
8. A time burning railway signal fusee containing sulfur and a perchlorate, said fusee having two sections both containing said ingredients in commingled condition, 130

but containing differing proportions of one of said ingredients, and therefore burnable with differing degrees of force and rapidity.

8. A time burning railway signal fusee  
5 containing metallic salt, sulfur and per-  
chlorate of potassium, a short portion of  
said fusee at the igniting end having said  
ingredients commingled, at least one of said  
latter two ingredients being contained there-  
10 in in excess thereby to cause the burning of  
said portion with excessive or abnormal

force and rapidity, and the remainder of  
said fusee having said ingredients normally  
proportioned, thereby to burn with less  
force and brilliancy.

In testimony whereof, I have signed my  
name to this specification, in the presence  
of two subscribing witnesses.

LOUIS S. ROSS.

Witnesses:

ROBERT H. KAMMLER,  
T. IRENE CHANDLER.